

## UNITED STATES PATENT OFFICE

2,192,984

## TREATMENT OF TEXTILE FABRICS

Henry Charles Olpin and George Holland Ellis,  
Spondon, near Derby, England, assignors to  
Celanese Corporation of America, a corporation  
of Delaware

No Drawing. Application March 29, 1938, Serial  
No. 198,686. In Great Britain April 9, 1937

13 Claims. (Cl. 8—15)

This invention relates to the treatment of textile fabrics, and particularly to the production of coloured effects on textile fabrics containing yarns of cellulose acetate or other organic derivatives of cellulose.

In U. S. applications S. Nos. 39,288, 39,289 and 39,290 filed 5th September, 1935, processes are described wherein filaments, yarns, fabrics and similar materials having a basis of organic derivatives of cellulose are subjected to esterification.

10 Thus, for example, filaments, yarns or fabrics having a basis of cellulose acetate may be subjected to an acetylation treatment. As indicated in the said specifications, the materials so produced have, in general, a somewhat reduced affinity for the dyestuffs commonly employed in dyeing cellulose acetate materials so that it is possible to produce cross-dyed effects by associating together in a fabric ordinary yarns of organic derivatives of cellulose and yarns of organic derivatives of cellulose which have been esterified, and dyeing the fabric with the ordinary dyestuffs used for cellulose acetate materials. The result is to produce a fabric in which the two types of 15 yarn are dyed to different depths, the ordinary yarn of organic derivative of cellulose being dyed the deeper shade.

It has now been discovered that certain classes of dyestuffs which have affinity for ordinary yarns of organic derivatives of cellulose have little or no affinity for yarns of organic derivatives of cellulose which have been esterified and that, in consequence, by treating with such dyestuffs fabrics which contain both ordinary yarns of organic 20 derivatives of cellulose and yarns of organic derivatives of cellulose which have been esterified products may be obtained in which the ordinary yarns are coloured and the esterified yarns are uncoloured by the treatment.

40 The invention is of greatest importance in connection with the production of fabrics exhibiting coloured effects where the fabrics contain yarns of cellulose acetate of acetyl content 52—55% (the ordinary acetate silk of commerce), and also yarns of this character which have been subjected to acetylation by one of the processes of the above-mentioned specifications, and the invention will therefore be described with particular reference to the treatment of such fabrics.

50 The dyestuffs found to be of value for the purpose of this invention are dyestuffs which have affinity for yarns of cellulose acetate of 52—55% acetyl content and which contain hydrophilic groups which do not possess in the dyestuffs in question any strong auxochromic effect. Of par-

ticular value are dyestuffs of this type which are sufficiently soluble in water to permit of their being applied from aqueous solution. As examples of hydrophilic groups there may be mentioned sulphonic acid groups, sulphuric acid ester groups, aliphatic hydroxy groups and carboxyl groups. In general the dyestuffs should not contain more than one sulphonic acid, sulphuric acid ester or carboxyl group, though in the case of dyestuffs containing aliphatic hydroxy groups two or more of such groups are permissible. As examples of suitable dyestuffs containing a sulphonic acid group there may be mentioned 1-amino-4-phenylamino-anthraquinone-2-sulphonic acid, 4'-(2:4-dinitrophenylamino)-4-methyl-diphenylamine - 6' - sulphonic acid, 2:6 - dinitro - benzene - 4 - sulphonic acid-azo- $\beta$ -naphthylamine, and 4-nitro-2- $\omega$ -sulpho - methyl - benzene-azo - ethylbenzylaniline. Suitable dyestuffs containing aliphatic hydroxy groups are, for example, anthraquinone dyestuffs 20 containing nuclear hydroxyalkyl, hydroxyalkyl-oxyl, or hydroxyalkylamino groups and azo dyestuffs obtained by diazotising aniline or its homologues, or their nitro or halogen substitution products, and coupling the diazotised compounds so 25 obtained with amino coupling components containing hydroxyalkyl groups, for example amino coupling components in which the amino group is substituted by an hydroxyalkyl group and an alkyl group. As examples of such dyestuffs there 30 may be mentioned 1:4 - diethanolamino - anthraquinone and 1:4-diethanolamino-5-hydroxy-anthraquinone. Suitable dyestuffs containing sulphuric acid ester groups are the sulphuric acid esters of dyestuffs containing single aliphatic hydroxy groups. As examples there may be mentioned the sulphuric acid esters of 1-methylamino-4-ethanolamino-anthraquinone, of 4-nitro-benzene-azo-ethyl - hydroxyethyl - aniline and of 4-nitro-2-chlorbenzene-azo-ethyl-hydroxyethyl-aniline.

35 The dyeing is preferably effected by treatment of the fabric with an aqueous dye liquor at a temperature below the boiling point of the liquor, e. g. at a temperature not above about 80° C. and 40 it is preferable that the conditions should be such that no substantial swelling of the esterified yarns takes place.

The fabric treated according to this invention 50 may contain the ordinary yarns of organic derivatives of cellulose, and yarns of organic derivatives of cellulose which have been esterified, associated together in any way. Thus, for example, the warp yarns, or part of the warp yarns, may be ordinary yarns of organic derivatives of 55

cellulose, and the weft yarns, or part of the weft yarns, may be yarns of organic derivatives of cellulose which have been esterified, or vice versa. The two types of yarn may be associated together

- 5 so that one type of yarn forms any desired pattern on a background of the other type of yarn. Again, the fabric may be formed from ordinary yarns of organic derivatives of cellulose and subjected to a process of local esterification in any  
10 desired pattern. Or, again, the fabric may contain mixed yarns which contain some ordinary filaments of organic derivatives of cellulose and some filaments of organic derivatives of cellulose which have been subjected to esterification, e. g.  
15 doubled yarns of which one constituent yarn is an ordinary organic derivative of cellulose yarn and the other is an organic derivative of cellulose yarn which has been subjected to esterification.

The esterified yarn present in the fabric may  
20 have been esterified by any suitable process. Of particular value, however, are yarns produced by the processes described in the specifications referred to above. The esterified yarn should be, or should approximate to, a tri-substitution product  
25 of cellulose. For example, in the case of acetylated cellulose acetate yarn the product should have an acetyl value of 59% or 60% or more, calculated as acetic acid.

The process of the invention may be modified,  
30 if desired, so that the esterified yarns of organic derivatives of cellulose in the final product, instead of being white, are also coloured. One way of achieving this result is to dye the esterified yarns of organic derivatives of cellulose  
35 with a suitable dyestuff before converting them into the fabric. Another way is to subject the esterified yarns to a process of superficial saponification before converting them into a fabric. In this way the esterified yarns, while still remaining unaffected by the dyestuffs used for  
40 colouring the ordinary yarns of organic derivatives of cellulose, acquire an affinity for direct dyestuffs, e. g. the dyestuffs commonly employed in the manufacture of cotton. Thus, for example,  
45 a fabric formed by associating together ordinary yarns of organic derivatives of cellulose and yarns of organic derivatives of cellulose which have been esterified and superficially saponified may be treated with a dyestuff of the type indicated above which will colour the ordinary yarns of organic derivatives of cellulose without colouring the esterified yarns, and also with a cotton dyestuff in order to colour the esterified and superficially saponified yarns. These dyestuffs  
50 may be applied in either order or simultaneously. The following example illustrates the invention but is not to be regarded as limiting it in any way:

*Example*

- 60 A fabric containing yarns of cellulose acetate of 52-54% acetyl content, and also similar yarns which have been acetylated by one of the processes of the specifications referred to above to an acetyl value of 60-62.5%, is immersed in an aqueous bath which is 30 times the weight of the fabric treated and which contains 40% of sodium sulphate on the weight of the fabric treated and 1% of 4'-(2:4-dinitrophenylamino)-  
65 4-methyl-diphenylamine-6'-sulphonic acid on the weight of the fabric treated. The dye bath is maintained at 80° C. After dyeing is completed the fabric is scoured and dried. The yarns of cellulose acetate of 52-54% acetyl content are dyed a good yellow shade while the  
70  
75

yarns which have been acetylated are uncoloured.

Similar results are obtained by substituting for the dyestuff used in this example one of the following dyestuffs:

The sulphuric acid ester of 4-nitro-benzene-azo-ethyl-hydroxyethyl-aniline; the sulphuric acid ester of 4-nitro-2-chlor-benzene-azo-ethyl-hydroxyethyl-aniline; 1 - amino-4-phenylamino-anthroquinone-2-sulphonic-acid.

Having described our invention what we desire to secure by Letters Patent is:

1. Process for the production of fabrics exhibiting colored effects, which comprises treating a fabric containing both yarns of cellulose acetate of acetyl value 52-55%, calculated as acetic acid, and similar yarns which have been esterified to an acidyl value corresponding to 2.7-3 acidyl radicles per  $C_6H_{10}O_5$  unit, so as to effect coloration of the former yarns without effecting any substantial coloration of the latter yarns with the dyestuff for the former yarns, by subjecting said fabric to the action of a dye liquid containing a dyestuff which has affinity for the former yarns and which contains a hydrophile group which has no strong auxochromic effect in the dyestuff.

2. Process for the production of fabrics exhibiting colored effects, which comprises treating a fabric containing both yarns of cellulose acetate of acetyl value 52 to 55% calculated as acetic acid and similar yarns which have been esterified to an acidyl value corresponding to 2.7 to 3 acidyl radicles per  $C_6H_{10}O_5$  unit, so as to effect coloration of the former yarns without effecting any substantial coloration of the latter yarns with the dyestuff for the former yarns, by subjecting said fabric to the action of a dye liquid containing a water-soluble dyestuff which has affinity for the former yarns and which contains a hydrophile group which has no strong auxochromic effect in the dyestuff.

3. Process for the production of fabrics exhibiting colored effects, which comprises treating a fabric containing both yarns of cellulose acetate of acetyl value 52 to 55% calculated as acetic acid and similar yarns which have been esterified to an acidyl value corresponding to 2.7 to 3 acidyl radicles per  $C_6H_{10}O_5$  unit, so as to effect coloration of the former yarns without effecting any substantial coloration of the latter yarns with the dyestuff for the former yarns, by subjecting said fabric to the action of a dye liquid containing a dyestuff which has affinity for the former yarns and which contains a single group containing the radicle  $-SO_2OH$ .

4. Process for the production of fabrics exhibiting colored effects, which comprises treating a fabric containing both yarns of cellulose acetate of acetyl value 52 to 55% calculated as acetic acid and similar yarns which have been esterified to an acidyl value corresponding to 2.7 to 3 acidyl radicles per  $C_6H_{10}O_5$  unit, so as to effect coloration of the former yarns without effecting any substantial coloration of the latter yarns with the dyestuff for the former yarns, by subjecting said fabric to the action of a dye liquid containing a dyestuff which has affinity for the former yarns and which contains a single sulphuric acid ester group.

5. Process for the production of fabrics exhibiting colored effects, which comprises treating a fabric containing both yarns of cellulose acetate of acetyl value 52 to 55% calculated as acetic acid and similar yarns which have been

- esterified to an acidyl value corresponding to 2.7 to 3 acidyl radicles per  $C_6H_{10}O_5$  unit, so as to effect coloration of the former yarns without effecting any substantial coloration of the latter 5 yarns with the dyestuff for the former yarns, by subjecting said fabric to the action of a dye liquid containing a dyestuff which has affinity for the former yarns and which contains at least two aliphatic hydroxy groups.
10. Process for the production of fabrics exhibiting colored effects, which comprises treating, at a temperature which is at most about 80° C., a fabric containing both yarns of cellulose acetate of acetyl value 52 to 55% calculated as 10 acetic acid and similar yarns which have been esterified to an acidyl value corresponding to 2.7 to 3 acidyl radicles per  $C_6H_{10}O_5$  unit, so as to effect coloration of the former yarns without effecting any substantial coloration of the latter 15 yarns with the dyestuff for the former yarns, by subjecting said fabric to the action of a dye liquid containing a dyestuff which has affinity for the former yarns and which contains a hydrophile group which has no strong auxochromic 20 effect in the dyestuff.
15. Process for the production of fabrics exhibiting colored effects, which comprises treating, at a temperature which is at most about 80° C., a fabric containing both yarns of cellulose acetate of acetyl value 52-55%, calculated as acetic acid, and similar yarns which have been esterified to an acidyl value corresponding to 2.7-3 acidyl radicles per  $C_6H_{10}O_5$  unit and subsequently 25 superficially saponified, so as to effect coloration of the former yarns without effecting any substantial coloration of the latter yarns with the dyestuff for the former yarns, by subjecting said fabric to the action of a dye liquid containing a dyestuff which has affinity for the former yarns and which contains a hydrophile group which has no strong auxochromic 30 effect in the dyestuff.
20. Process for the production of fabrics exhibiting colored effects, which comprises treating, at a temperature of at most about 80° C., a fabric containing both yarns of cellulose acetate of acetyl value 52-55%, calculated as acetic acid, and similar yarns which have been esterified to an acidyl value corresponding to 2.7-3 acidyl radicles per  $C_6H_{10}O_5$  unit and subsequently 35 superficially saponified, so as to effect coloration of the former yarns without effecting any substantial coloration of the latter yarns with the dyestuff for the former yarns, by subjecting said fabric to the action of a dye liquid containing a water-soluble dyestuff which has affinity for the former yarns and which contains a hydrophile group which has no strong auxochromic 40 effect in the dyestuff.
25. Process for the production of fabrics exhibiting colored effects, which comprises treating a fabric containing both yarns of cellulose acetate of acetyl value 52-55%, calculated as acetic acid, and similar yarns which have been esterified to an acidyl value corresponding to 2.7-3 acidyl radicles per  $C_6H_{10}O_5$  radicle and colored before being incorporated in the fabric, so as to effect 45 coloration of the former yarns without effecting any substantial coloration of the latter yarns with the dyestuff for the former yarns, by subjecting said fabric to the action of a dye liquid containing a dyestuff which has affinity for the former yarns and which contains a hydrophile group which has no strong auxochromic 50 effect in the dyestuff.

30. Process for the production of fabrics exhibiting colored effects, which comprises treating a fabric containing both yarns of an organic derivative of cellulose which is soluble in organic solvents and similar yarns which have been esterified until they contain from 2.7 to 3 substituent radicles per  $C_6H_{10}O_5$  unit so as to effect coloration of the former yarns without effecting 55 any substantial coloration of the latter yarns with the dyestuff for the former yarns, by subjecting said fabric to the action of a dye liquid containing a dyestuff which has affinity for the former yarns and which contains a hydrophile group which has no strong auxochromic 60 effect in the dyestuff.

35. Process for the production of fabrics exhibiting colored effects, which comprises treating a fabric containing both yarns of an organic derivative of cellulose which is soluble in organic solvents and similar yarns which have been esterified to an acidyl value corresponding to 2.7 to 3 acidyl radicles per  $C_6H_{10}O_5$  unit and subsequently 65 superficially saponified, so as to effect coloration of the former yarns without effecting any substantial coloration of the latter yarns with the dyestuff for the former yarns, by sub-

jecting said fabric to the action of a dye liquid containing a dyestuff which has affinity for the former yarns and which contains a hydrophile group which has no strong auxochromic effect in the dyestuff.

40. Process for the production of fabrics exhibiting colored effects, which comprises treating a fabric containing both yarns of cellulose acetate of acetyl value 52-55%, calculated as acetic acid, and similar yarns which have been esterified to an acidyl value corresponding to 2.7 to 3 acidyl radicles per  $C_6H_{10}O_5$  unit and subsequently 45 superficially saponified, so as to effect coloration of the former yarns without effecting any substantial coloration of the latter yarns with the dyestuff for the former yarns, by subjecting said fabric to the action of a dye liquid containing a dyestuff which has affinity for the former yarns and which contains a hydrophile group which has no strong auxochromic 50 effect in the dyestuff.

45. Process for the production of fabrics exhibiting colored effects, which comprises treating a fabric containing both yarns of cellulose acetate of acetyl value 52-55%, calculated as acetic acid, and similar yarns which have been esterified to an acidyl value corresponding to 2.7-3 acidyl radicles per  $C_6H_{10}O_5$  unit and subsequently 55 superficially saponified, so as to effect coloration of the former yarns without effecting any substantial coloration of the latter yarns with the dyestuff for the former yarns, by subjecting said fabric to the action of a dye liquid containing a water-soluble dyestuff which has affinity for the former yarns and which contains a hydrophile group which has no strong auxochromic 60 effect in the dyestuff.

50. Process for the production of fabrics exhibiting colored effects which comprises treating a fabric containing both yarns of an organic derivative of cellulose which is soluble in organic solvents and similar yarns which have been esterified until they contain from 2.7 to 3 substituent radicles per  $C_6H_{10}O_5$  unit so as to effect coloration of the former yarns without effecting 65 any substantial coloration of the latter yarns with the dyestuff for the former yarns, by subjecting said fabric to the action of a dye liquid containing a dyestuff which has affinity for the former yarns and which contains a hydrophile group which has no strong auxochromic 70 effect in the dyestuff.

55. Process for the production of fabrics exhibiting colored effects, which comprises treating a fabric containing both yarns of acetone-soluble cellulose acetate and similar yarns which have been esterified to an acidyl value corresponding to 2.7 to 3 acidyl radicles per  $C_6H_{10}O_5$  unit, so as to effect coloration of the former yarns without effecting any substantial coloration of the latter yarns with the dyestuff for the former yarns, by subjecting said fabric to the action of a dye liquid containing a dyestuff which has affinity for the former yarns and which contains a hydrophile group which has no strong auxochromic 80 effect in the dyestuff.

HENRY CHARLES OLPIN.  
GEORGE HOLLAND ELLIS.